

## UNITED STATES PATENT OFFICE

2,239,869

## PROCESS FOR TREATING LIQUID ZINC AMALGAMS

Hermann Wolf, Ernst Kuss, Hans Hohn, and Fritz Stietzel, Duisburg Germany, assignors of one-half to Duisburger Kupferhütte, Duisburg, Germany, and one-half to I. G. Farbenindustrie Aktiengesellschaft, Frankfort - on - the - Main, Germany

No Drawing. Application August 11, 1939, Serial No. 289,632. In Germany June 21, 1937

9 Claims. (Cl. 75—97)

The present invention relates to a process for maintaining the good flowability of liquid zinc amalgams.

For the technical working with zinc amalgams it is necessary, if desired to cause the amalgam to circulate, to pass it through tubes and exactly to proportion its proportions, such steps and the performance of continuous processes in general require a good fluidity (i. e. mobility) of the zinc amalgam. Such good fluidity especially is also required when preparing the amalgams electrolytically. It has been attempted to produce this desirable fluidity by working in an inert gas, especially in a nitrogen atmosphere so as to prevent the formation of oxide.

In accordance with the present invention the good flowability of zinc amalgams can be maintained in an especially advantageous manner, with certainty and permanently, by bringing into contact the zinc amalgams with solutions having the property of dissolving zinc oxide, preferably with aqueous solutions and of such concentration that the zinc amalgam is practically not attacked. The working may be performed at ordinary or higher temperatures. In most cases it is advantageous to cover the amalgam with solutions; amalgam, for instance, which has been manufactured in a horizontal cell as is used in the chlorine alkali electrolysis, and which is passed back into the cycle from the cell to the circulation pump by way of a return channel, is brought into contact with solutions in such a way that the solvent is injected into the pumps and then is led back through a channel, whereupon the amalgam is covered by the solutions. It is especially advantageous to use aqueous dilute hydrochloric or sulfuric acid solutions; for example  $\frac{1}{2}$  normal hydrochloric acid solutions may be used. But it is also possible to use alkaline reacting solutions, as for instance ammonia and ammonium carbonate solutions. Furthermore solutions may be used containing free chlorine. The dilute aqueous solutions used take up only such a small quantity of zinc that it may be neglected when compared with the content of zinc of the amalgams. Preferably the solution is passed over the amalgam in a slow stream, so that the solution is continuously renewed. It is also possible to use anhydrous, for instance ethereal and alcoholic solutions, for instance such solutions of hydrogen chloride or bromide. Amalgams already oxidized acquire good fluidity again when treated with solutions in accordance with the process mentioned above.

The invention is further illustrated in the following examples:

*Example 1*

In one of the known amalgam cells, as generally used in the industry for electrolyzing alkali metal chlorides, of a width of  $\frac{1}{2}$  meter and a length of about 6 meters, mercury flowing at the bottom of the cell from one end to the other below the electrolyte serves as the cathode. The amalgam formed flows back from a considerably narrower return channel to the other end, and is then fed by means of a circulating pump back into the cell proper, so that an interrupted circuit of the mercury or amalgam respectively takes place. From the amalgam continuously circulating a part of the zinc amalgam corresponding to the electrical current is permanently taken off and worked up in the desired manner, while at the other end continuously a corresponding quantity of fresh mercury is fed in.

In that part of the cell not passed by the current the amalgam is irrigated by a  $\frac{1}{2}$  normal aqueous hydrochloric acid heated to  $90^{\circ}$  C. The acid is injected for this purpose into the inner part of the circulating pump when it overflows into the return channel; it then flows through the whole length of the channel and leaves it at the other end through an overflow. The speed of feeding amounts to 30-60 liters per hour. The success of this procedure is such a perfect one that after 3 months of working the amalgam is still as bright as it was before. This result is obtained without filling the apparatus with inert gases. The exclusion of oxygen has proved superfluous.

*Example 2*

The working is performed as described in Example 1, but for irrigation of the amalgam an electrolyte weakly acidified with sulfuric acid is chosen. Above the position where the hot electrolyte flows into that part of the cell conducting the current a part is taken off and introduced together with a small quantity of sulfuric acid into the circulating pump. The content of sulfuric acid of the electrolyte thus introduced amounts to  $\frac{1}{20}$  normal. After a few days in this case also the amalgam remains absolutely bright.

*Example 3*

In a trough, provided with a scoop apparatus and closed against the outer air a 5% amalgam heated up to  $75^{\circ}$  C. flows for concentration purposes. Through the same trough flows a 4-nor-

mal ammonium carbonate solution cooled to +5° C., which is circulated by a pump between this trough and a heat exchanger. By means of the scoop apparatus a kneadable solid amalgam with an average zinc content of 10% is drawn off while an about 1½% readily mobile amalgam flows away through an overflow. The ammonium carbonate solution enriched with zinc is removed from time to time, about once a week, the ammonium carbonate regenerated by driving off with steam and introducing carbonic acid, and the basic zinc carbonate resulting therefrom is obtained as a by-product.

*Example 4*

The working is performed as described in Example 1 while using instead of the hydrochloric acid the electrolyte running off from that part of the cell conducting the current and containing free chlorine.

*Example 5*

An apparatus for the distillation of zinc amalgam is fed from a cast-iron vessel in which a 5% zinc amalgam, heated to 75° C. is covered by a 10% sodium hydroxide solution; the sodium hydroxide solution is drawn off from time to time and replaced by a fresh one.

*Example 6*

In front of a valve destined for measuring the zinc amalgam a cylindrical vessel is located provided with a siphon delivery. The amalgam present in the vessel is covered with water, through which a part of the chlorine gas evolved in the cell is slowly passed.

*Example 7*

In front of a valve destined for measuring the zinc amalgam a cylindrical vessel is located provided with a siphon delivery. The amalgam contained in the vessel is covered with 1 normal ethereal hydrochloric acid.

This application is a "continuation-in-part" to our copending application Ser No. 214,954, filed June 21, 1938.

We claim:

1. Process for maintaining the good flowability of liquid zinc amalgam which consists in covering the liquid zinc amalgam with solutions of substances capable of dissolving zinc oxide and of such a concentration that the zinc amalgam is practically not attacked.

2. Process for maintaining the good flowability

of liquid zinc amalgam which consists in covering the liquid zinc amalgam with aqueous solutions of substances capable of dissolving zinc oxide and of such a concentration that the zinc amalgam is practically not attacked.

3. Process for maintaining the good flowability of liquid zinc amalgam which consists in covering the liquid zinc amalgam with acid reacting aqueous solutions of substances capable of dissolving zinc oxide and of such a concentration that the zinc amalgam is practically not attacked.

4. Process for maintaining the good flowability of liquid zinc amalgam which consists in covering the liquid zinc amalgam with aqueous solutions of hydrochloric acid capable of dissolving zinc oxide and of such a concentration that the zinc amalgam is practically not attacked.

5. Process for maintaining the good flowability of liquid zinc amalgam which consists in covering the liquid zinc amalgam with basic reacting aqueous solutions of substances capable of dissolving zinc oxide and of such a concentration that the zinc amalgam is practically not attacked.

6. Process for maintaining the good flowability of liquid zinc amalgam which consists in covering the liquid zinc amalgam with aqueous solutions of ammonium carbonate capable of dissolving zinc oxide and of such a concentration that the zinc amalgam is practically not attacked.

7. Process for maintaining the good flowability of liquid zinc amalgam which consists in covering the liquid zinc amalgam with organic solutions of substances capable of dissolving zinc oxide and of such a concentration that the zinc amalgam is practically not attacked.

8. Process for maintaining the good flowability of liquid zinc amalgam which consists in covering the liquid zinc amalgam with organic solutions of an acid capable of dissolving zinc oxide and of such a concentration that the zinc amalgam is practically not attacked.

9. Process for maintaining the good flowability of liquid zinc amalgam which consists in covering the liquid zinc amalgam with an alcoholic solution of hydrochloric acid capable of dissolving zinc oxide and of such a concentration that the zinc amalgam is practically not attacked.

HERMANN WOLF.  
ERNST KUSS.  
HANS HOHN.  
FRITZ STIETZEL.